

Jan. 16, 1923.

1,442,326.

J. DE LONG.  
INSULATING MATERIAL AND PROCESS OF MANUFACTURING SAME.  
FILED NOV. 26, 1921.

*Fig. 1*



*Fig. 2*



*Julius De Long* *INVENTOR*  
*Henry M. Daubens* *BY* *his ATTORNEY*

Patented Jan. 16, 1923.

1,442,326

# UNITED STATES PATENT OFFICE.

JULIUS DE LONG, OF LAKE MAHOPAC, NEW YORK.

## INSULATING MATERIAL AND PROCESS OF MANUFACTURING SAME.

Application filed November 26, 1921. Serial No. 517,923.

To all whom it may concern:

Be it known that I, JULIUS DE LONG, a citizen of the United States, residing at Lake Mahopac, in the county of Putnam and State of New York, have invented new and useful Improvements in Insulating Materials and Processes of Manufacturing Same, of which the following is a specification.

10 My invention relates to improvements in insulating material which are particularly adapted for use in insulating railroad cars, buildings and other structures, and the objects of my invention are to produce a new 15 insulating material which can be cheaply and economically manufactured, which will be essentially fireproof in its character, and which is a far better non-conductor of heat than the previous types of fireproof insulating material heretofore in use, and which also possesses sufficient rigidity to be easily handled and applied. Reference is hereby made to the following pending applications by the applicant relating to the same or kindred subject matter, namely: Serial No. 25 432,649, Serial No. 556,579, and Serial No. 591,362.

Figure 1 is a perspective view of my insulating material with the layers of the material used partly broken away.

Figure 2 is an enlarged sectional view on the line XX of Figure 1.

In the drawings, 1 indicates the woven fabric; 2 the bats of asbestos fibre and cattle hair, and 3 the covering of asbestos paper.

Heretofore fireproof insulating material has been made from asbestos fibre, but in this type of insulating material the fibres 40 were always secured together by glue or other adhesive material which tended to close and fill the air spaces between the fibre and thereby greatly decrease the insulating value of such insulating material.

45 Insulating material has also been formed by mingling asbestos fibre and cattle hair, but in the past these fibres have also been secured together by means of glue or other adhesive material which tended to fill the 50 air spaces between the fibres and detracted from the insulating value of the material so formed. Material so formed is also liable to disintegrate and fall apart when damp or wet and therefore is undesirable for many 55 purposes for which insulating material is used.

I have found that I can make a strong, durable insulating material by the following process:

I run finely divided asbestos fibre and cattle hair through a picker and form the commingled asbestos fibre and cattle hair into bats by running it through a carding machine. I lay a bat so formed upon a strip of burlap or other suitable woven fabric 60 possessing the desired strength, and run the bat and burlap through a punching needle loom, said needles forcing the asbestos fibre and cattle hair through the burlap and interlocking the fibres of asbestos and cattle 65 hair with each other and firmly securing the bat to the burlap or other woven material. When this operation is completed, I turn the product over and place another similarly formed bat upon the exposed surface of the 70 burlap or other woven fabric and again run the material through the punching needle loom with the result that the fibres of asbestos and cattle hair in the upper bat are interlocked and the fibres from the upper 75 bat are driven through the burlap or other woven fabric, and more or less interlocked with the asbestos fibre and cattle hair on the opposite side of the burlap or other woven fabric. This produces a strong, durable 80 felt which is a far better nonconductor of heat than the material heretofore used and is at the same time essentially fireproof. I prefer to use equal quantities of asbestos fibre and cattle hair, as this produces a material which is fireproof, strong 85 and durable. These proportions may, however, be varied without departing from the spirit of my invention.

Where a rigid material is required, I apply adhesive material to the surface of asbestos paper or other suitable covering, which I apply to one or both of the outer surfaces of the felt formed as above stated. 90 Where asbestos paper is so applied, and particularly when it is applied to both sides of the felt, the insulating value is increased because of the dead air trapped between the sheets of asbestos paper, and the material possesses sufficient rigidity and strength to 100 be easily handled and applied.

Having described my invention, I claim:

1. An insulating material comprising in combination woven fabric, bats composed of asbestos fibre and cattle hair on each side 110 of said woven fabric, the cattle hair and asbestos fibre in each bat being interlocked

with each other, with the woven fabric and with the asbestos fibre and cattle hair of the bat on the opposite side of such woven fabric.

2. An insulating material comprising in combination woven fabric, bats composed of asbestos fibre and cattle hair on each side of said woven fabric, the cattle hair and asbestos fibre in each bat being interlocked with each other, with the woven fabric and with the asbestos fibre and cattle hair of the bat on the opposite side of such woven fabric, and an asbestos covering on each side thereof and secured thereto by adhesive material.
3. An insulating material comprising in combination woven fabric, bats composed of asbestos fibre and cattle hair arranged on opposite sides of such woven fabric and secured to each other and to such woven fabric by interlocking the asbestos fibre and cattle hair of each bat with the asbestos fibre and cattle hair of the other bat and with such woven fabric.
4. An insulating material comprising in combination woven fabric, bats composed of

asbestos fibre and cattle hair arranged on opposite sides of such woven fabric and secured to each other and to such woven fabric by interlocking the asbestos fibre and cattle hair of each bat with the asbestos fibre and cattle hair of the other bat and with such woven fabric, and an asbestos covering on each side thereof and secured thereto by adhesive material.

5. The process of making insulating material consisting of (1) passing asbestos fibre and cattle hair through a picking machine, (2) forming the product thus obtained into a bat by passing the same through a carding machine, (3) arranging the bat so formed on woven material and securing the bat to the woven material by passing both through a punching needle loom, (4) placing a bat formed as above stated on the opposite side of the woven fabric and running the same through a punching needle loom.

Signed at New York, this 25th day of November, 1921.

JULIUS DE LONG.